

## UNITED STATES PATENT OFFICE

FREDERICK M. BECKET, OF NEW YORK, N. Y.

## PROCESS OF MAKING IRON-CHROMIUM NICKEL ALLOYS

No Drawing.

Application filed November 18, 1930. Serial No. 496,569.

The invention is a process of making alloys containing iron, chromium and nickel, with or without other metals. The object of the invention is to make such alloys more economically than by the methods heretofore practised. This object is attained by using relatively inexpensive sources of nickel and chromium, viz., nickel matte, and high- or medium-carbon ferrochrome.

10 I have found that by furnacing nickel matte under appropriate conditions with high carbon ferrochrome, which is the least expensive form of metallic chromium now available, the sulphur of the matte can be almost quantitatively expelled, and at least a part of the carbon in the ferrochrome simultaneously eliminated. The resulting alloy, containing the nickel of the matte together with the iron and chromium of the ferrochrome, and more or less carbon, is useful for many purposes, either as produced, or after further treatment. For example, the alloy can be diluted with iron to produce steels of the stainless type. In making stain-  
25 less steel by the process of my invention, I prefer to carry out the reaction between the carbon of the ferrochrome and the nickel sulphide of the matte in such manner that the ratio of carbon to chromium in the alloy thereby produced will be somewhat higher than is preferred in stainless steels; and to remove some of the carbon in a subsequent operation, as by treating the metal with an oxidizing slag, or Bessemerizing it with commercial oxygen or air strongly enriched with oxygen. If the further treatment of the initial alloy comprises dilution with iron, the decarburizing operation can be applied either before or after such dilution.

40 I prefer to compound the charge in such manner that somewhat more than one atom of carbon to two of sulphur will be present, the 1 to 2 ratio being that in which the elements combine to form carbon disulphide. An excess of carbon favors a more complete elimination of sulphur, but it will be understood that a complete expulsion of sulphur is unnecessary, and is in general impossible in ferrous metallurgy; and any proportion of carbon which will give a useful product is

within my invention. In this connection it may be remarked that sulphur will usually be in some degree eliminated in the decarburizing and refining treatments to which the initial alloy will normally be subjected, while mere dilution of the initial alloy with low-sulphur iron will of course lower the percentage of sulphur.

Since the permissible variation in the ratio of carbon to sulphur is a wide one, and since the ratio of chromium to carbon in ferrochromes can be varied through a considerable range without materially increasing the cost per pound of contained chromium, the ratio of chromium to nickel in the initial alloy can be readily controlled. As will be shown in a specific example given below, it is possible so to make up the charge that after the initial alloy is refined and decarburized with the loss of some chromium, the chromium-to-nickel ratio in the final product can be made to fall at about  $2\frac{1}{4}$  to 1, the ratio in the common 18% chromium-8% nickel stainless steel.

75 In carrying out the process, the finely ground materials are preferably charged into an electric smelting furnace of the open-arc type at a rate commensurate with the rate of reaction. For best results as regards completeness of reaction it is desirable to operate at as high a temperature as the refractory lining of the furnace will allow. I prefer to have some lime in the charge as a slag-forming material, and it is usually advisable to employ some fluorspar in the mix-  
80 ture to impart fluidity to the slag.

85 In the preferred embodiment of my invention, a ferrochrome-nickel alloy containing between one and two per cent of carbon is produced in the initial stage. The alloy is then transferred to a Bessemer converter and blown preferably with commercially pure oxygen or highly oxygenated air until the carbon has been reduced to the desired point.

90 Below are given examples to show the results attainable by the above-described process:

*Example I*

One hundred parts of high-carbon ferrochrome, 50 parts of nickel matte, 50 parts of

lime and 25 parts of fluorspar were mixed and charged gradually into an open-arc electric furnace which contained a small bath of molten slag made up with lime and silica in 5 the ratio of 3 parts of lime to 1 part of quartzite. The high-carbon ferrochrome contained 69.71% chromium, 1.37% silicon and 4.89% carbon, and was smaller than 8 mesh. The nickel matte contained 75.28% 10 nickel and 23.70% sulphur, and was also below 8 mesh in size. The lime and fluorspar were of the usual commercial grades. The product, ferrochrome-nickel, analyzed:

|                        | Per cent |
|------------------------|----------|
| 15 Chromium            | 47.03    |
| Nickel                 | 28.52    |
| Carbon                 | 1.82     |
| Silicon                | 0.07     |
| Sulphur                | 0.08     |
| 20 Balance mostly iron |          |

### Example II

In another run the following mixture was charged onto a small molten bath made up 25 with lime and silica in the ratio of two parts of lime to one part of quartzite:

|                         | Parts |
|-------------------------|-------|
| High-carbon ferrochrome | 450   |
| Nickel matte            | 112   |
| 30 Lime                 | 185   |
| Fluorspar               | 30    |

The high-carbon ferrochrome, sized smaller than 8 mesh, contained 68.23% chromium, 4.96% carbon and 1.51% silicon. The nickel 35 matte, also sized smaller than 8 mesh, contained 74.90% nickel and 23.71% sulphur. The lime and fluorspar were of the usual commercial grade. The above mixture was charged at a uniform rate, and the furnace 40 used was an open-arc electric furnace operating at a high temperature. Upon completion of the smelting, a sample of the alloy was taken which analyzed as follows:

| 45 | Percent Cr | Percent Ni | Percent Fe | Percent C | Percent Si | Percent S |
|----|------------|------------|------------|-----------|------------|-----------|
|    | 56.46      | 17.24      | 23.56      | 1.77      | 0.10       | 0.049     |

50 The molten alloy was tapped directly into a Bessemer converter and blown for 30 minutes with a blast of commercially pure oxygen. Upon completion of the blow the alloy was cast in pig form. Analysis of the final 55 product showed:

| 50 | Percent Cr | Percent Ni | Percent Fe | Percent C | Percent Si | Percent S |
|----|------------|------------|------------|-----------|------------|-----------|
|    | 49.66      | 21.20      | 27.25      | 0.16      | 0.05       | 0.040     |

### Example III

The following example is illustrative of the process as applied to the manufacture 65 of stainless steel of the 18% chromium-8%

nickel variety. Materials making up the charge, proportioned as shown below, were of the same analysis and size as those employed in the immediately preceding example:

|                         | Parts |
|-------------------------|-------|
| High-carbon ferrochrome | 200   |
| Nickel matte            | 40    |
| Lime                    | 75    |
| Fluorspar               | 8     |
|                         | 75    |

The above mixture was charged into an open-arc electric furnace, operated at a high temperature, at a uniform rate. After completion of the smelting, 240 parts of steel scrap were melted into the alloy, which was thereupon tapped into a Bessemer converter and blown with commercially pure oxygen for 8½ minutes. From the converter, the steel was tapped into two ladles and then into ingot molds after treatment with 0.40% manganese as low carbon ferromanganese and 0.40% silicon as 50% ferrosilicon. The two ladles were separately analyzed, the average of the closely concordant analytical figures being as follows:

| Percent Cr | Percent Ni | Percent Si | Percent C | Percent Mn |
|------------|------------|------------|-----------|------------|
| 17.29      | 7.66       | 0.11       | 0.05      | 0.26       |

The average results of physical tests of the metal are shown below: The test pieces were quenched from 1150° C.

|                   |                          |     |
|-------------------|--------------------------|-----|
| Maximum stress    | 119,300 lbs. per sq. in. | 100 |
| Yield point       | 30,900 lbs. per sq. in.  |     |
| Elongation        | 38%                      |     |
| Reduction of area | 54%                      |     |
| Impact            | 80 ft. lbs.—break        |     |
| Erichsen value    | 10.8                     | 105 |
| Brinell hardness  | 131                      |     |

It is obvious that in cases where a higher carbon content is allowable than that of the steel produced in Example III, the blow may be shorter, with a resulting conservation of some of the chromium lost in the longer blow. In certain cases where the best possible physical properties are required, the molten alloy may be transferred from the converter to an electric steel furnace for finishing.

I claim:

1. A process of making alloys containing iron, chromium and nickel which comprises the step of reacting on nickel matte with carbon-containing ferrochrome in the presence of basic slag-forming material, the quantities of ferrochrome and matte used being such that the charge contains more than one carbon atom to each two sulphur atoms.

2. A process of making low-carbon low-sulphur alloys containing iron, chromium and nickel which comprises reacting on nickel matte with lime and an excess of carbon in

the form of carbon-containing ferrochrome, and thereafter oxidizing at least a part of the residual carbon by Bessemerization.

3. A process of making chrome-nickel stainless steel which comprises reacting on nickel matte with lime and an excess of carbon in the form of high-carbon ferrochrome, oxidizing at least a part of the residual carbon by Bessemerization, and adding iron to the alloy produced by the first-mentioned reaction.

4. A process of making stainless steel which comprises melting high-carbon ferrochrome with lime and nickel matte and heating the mixture until the sulphur is substantially eliminated and an alloy containing at least 1.0% of carbon is formed; raising the ratio of chromium to carbon to a value suitable for stainless steel by blowing the metal, 15 in the molten state, with commercially pure oxygen, and diluting the alloy with iron at any stage after the elimination of the sulphur.

5. The method of reducing nickel matte which comprises reacting on said matte, in 20 the presence of basic slag-forming material, with an excess of carbon in the form of carbon-containing ferrochrome.

6. The method of reducing nickel matte which comprises reacting on said matte with 25 lime and an excess of carbon, said carbon being in the form of high-carbon ferrochrome.

7. A process of making low-carbon low-sulphur alloys containing iron, chromium, 30 and nickel which comprises reacting on nickel matte, in the presence of basic slag-forming material, with an excess of carbon in the form of carbon-containing ferrochrome, and thereafter oxidizing at least a part of the 35 residual carbon.

8. A process of making chromium-nickel stainless steels which comprises reacting on nickel matte, in the presence of basic slag-forming material, with an excess of carbon 40 in the form of carbon containing ferrochrome, oxidizing at least a part of the residual carbon, and adding iron to the alloy produced by the last-mentioned reaction.

9. A process of making low-carbon low-sulphur alloys containing iron, chromium and nickel which comprises reacting on nickel matte, in the presence of basic slag-forming material, with an excess of carbon in the form of carbon-containing ferrochrome, and there- 45 after oxidizing at least a part of the residual carbon by Bessemerization.

10. A process of making chromium-nickel stainless steels which comprises reacting on nickel matte, in the presence of basic slag- 50 forming material, with an excess of carbon in the form of carbon-containing ferrochrome, and oxidizing at least a part of the residual carbon by blowing the metal in the molten state with oxygen-enriched air.

65 11. A process of making chromium-nickel

stainless steels which comprises reacting on nickel matte, in the presence of a basic slag, with an excess of carbon in the form or carbon-containing ferrochrome, and heating the mixture until the sulphur is substantially 70 eliminated and an alloy containing at least 1.0% of carbon is formed; raising the ratio of chromium to carbon to a value suitable for stainless steel by blowing the metal in the molten state with oxygen-enriched air, 75 and diluting the alloy with iron at any stage after the elimination of the sulphur.

In testimony whereof, I affix my signature.  
FREDERICK M. BECKET.